

## UNITED STATES PATENT OFFICE

2,157,206

## MANUFACTURE OF DIAZO TYPE MATERIAL

Walker M. Hinman, Winnetka, Ill., assignor to  
The Frederick Post Company, Chicago, Ill., a  
corporation of Illinois

No Drawing. Application January 6, 1937,  
Serial No. 119,288

## 2 Claims. (CL. 85—6)

The present invention relates to diazotypes and has particular relation to the appearance of the print with respect to changes in the background.

5 Diazotypes are positive prints made upon sensitized paper by the printing action of actinic light through a light transmitting pattern. A sensitizing substance is used which is capable of union with a coupling agent to create a dye-stuff. The sensitizing substance can be destroyed by light, so that where light strikes, no dye can form. The light-printed sensitized papers vary 10 in composition and may be developed in various ways, as by water, or by developer solution, or by ammonia vapors, and then dried. The fresh 15 dry print should have no color where it is struck by light, and hence on white paper should show a white field or background for a lined drawing. Under the influence of ordinary light acting for a long time, or of strong light acting for 20 a shorter time, a so-called discoloration appears as a yellowing or browning of the originally whiter field.

Various attempts have been made to avoid this 25 discoloration or so-called discoloration. One of these has been to use a reducing agent in the print. This is only partially effective, and quite suitable for ordinary uses, but not for strong sunlight. Other attempts have been made to mask 30 the color change by employing a paper made from dyed stock. In one instance a green paper was used, but when the coloration occurred the colored face and the green back were quite contrasting. But a white and not a colored background is commercially desired.

35 The present invention aims to avoid the effects of discoloration by masking the same, and to provide a white print lacking in severe contrast between its face and its back, when freshly made and when aged to the extent that it would appear 40 discolored if on a pure white stock.

The present invention takes advantage of the power of a light blue color to mask a yellow or tan on white, and to give the appearance of white.

45 The unqualified word "white" is not used in its true technical sense, which means a neutralizing mixture of all visible color, but rather in its commercial sense with reference to the color of so-called "white" papers. A white paper may be on the yellow, or the blue, or some other color, and yet be called a white paper. The character of "whiteness" is more apparent when comparing 50 side-by-side, two differently white papers. For example, the face of a slightly discolored diazo-type on a white stock may look white by itself, but when it is compared to the back of the print, it will appear pale yellow or tan. The exact color 55 may depend a great deal upon the residual chemicals left in the print, and these may vary with the character of the sensitizing solution, or the

character of the developer, or with the treatment of the print.

It has been observed that a blue-white is not so contrasting with a better white, as is a yellow-white. Therefore, the invention contemplates 5 using a stock which is white on one side and a bluer white on the sensitized side. When a print is dry and not discolored from the effect of light, the white back of the print is not highly contrasting with the bluer white face. Then as yellow or tan is produced on aging, the newly 10 formed color is "neutralized" by the blue which is present.

The above statement is perhaps merely a practical statement of the invention, which permits 15 the results to be understood. But it may not explain the mechanism. It is suggested that the action of the blue may not be entirely or partially one of neutralization, but rather one of filtering out or absorbing certain light rays or 20 fractions thereof which effect the discoloration.

As mentioned above a reducing agent may be used to minimize discoloration as set forth in the Van der Grinten U. S. Patent No. 1,821,281 and No. 1,841,653. In that patent it is set forth that the reducing agent may be added in one of numerous ways or in a combination of them. It may be present in the paper before coating, in the coating solution, in the developer, or be specially applied after the print is completed. The present invention may be used with or without a reducing agent which may be applied according to said patent. The combination use of blue and of reducing agent is more effective than use of the blue alone, or use of the reducing agent alone. The reducing agent retards the formation 30 of discoloring material, and the blue color masks it when and if it does form. A paper having reducing agent which may get yellow in strong sunlight, will appear less yellow if the blue is 35 present.

The invention may be carried out in numerous ways. The blue color may be impressed or applied to one side of the stock sheet to be sensitized, or laminated sheet stock may be used 45 with a white facing sheet and a bluer white facing sheet. The objective is to have the back side white, with the face a bluer white. The blue color may be applied in a sizing bath with which the stock may be sized on its face. Also the 50 blue color may be applied in the sensitizing solution. Developer solution or wash water may be used with blue color therein to apply the blue tint, and it may even be applied after the print is completed. Several of these ways may be used 55 in combination.

A preferred method of applying the blue color has been found. That is to apply it from the sensitizing solution. For the purpose of the present invention a blue dyestuff may be added 60

to the sensitizing solution to give a blue tint to the background of the finished print, for example enough Pontacyl Brilliant Blue 2R, made by E. I. du Pont de Nemours of Wilmington, Delaware, to make the bath about .04% in such dyestuff. This is coated directly onto the face of white paper stock and dried. The diazo solution may be colorless or colored, depending in one respect upon the color of the diazo component employed. Where a yellow diazo solution is used, the dried sensitized sheet looks white on the back and green on the coated face. Upon light-printing the face of the sheet becomes blue-tinted where struck by light, and remains green only where the image of the pattern lies. This green image may be strengthened by a developer.

The invention may be carried out as follows: An ordinary sensitizing bath may be used, such as one containing

|                                                 | Grams per liter |
|-------------------------------------------------|-----------------|
| Chlorostannate of para diazo di-n-butyl aniline | 20.0            |
| 25 Pontacyl Brilliant Blue 2R                   | 4               |
| Water.                                          |                 |

The solution is applied to one side of suitable stock and the coating dried. When printed by light, it may be developed by wetting in any well-known manner with a solution of

|                                | Grams per liter |
|--------------------------------|-----------------|
| Sodium carbonate (monohydrate) | 10              |
| Phloroglucinol                 | 4               |

35 The paper is merely wet with the developer, and it need not but may be washed afterwards. If the print is to be made more resistant to discoloration in strong light, reducing agent may be added as above mentioned. This may be conveniently done by adding 30 grams per liter of sodium thiosulphate to the above developer solution when the developed print is not to be washed. The dry print is then without strong contrast between its face and its back, and this close 40 identify of the back of the print and the background of the face continues and remains under conditions where the same print lacking the blue color would show a contrast between a white back and a discolored face.

45 50 It is preferred to apply the color in the sensitizing solution for several reasons. The color itself appears to be more permanent against fading in light, when it is applied from the sensitizing bath, than when it is applied directly to the paper before sensitizing. By this method the dye appears to be more a part of the chemicals than a part of the fiber. Hence it can be effective on chemicals lying between fibers or on fibers. Also it has been found that the blue 55 color applied from the sensitizing bath renders the unprinted sensitized sheet more stable for storage before use. It has better keeping qualities. Stored sensitized paper of the prior art does deteriorate and as it does so, it develops a tan color. This tan color is present in the background initially on printing and developing. These circumstances present again the question of whether the blue color acts chemically to prevent the discoloration on storage, or whether it physically masks to the human eye, the slight color which is formed, or whether it is both effects combined.

55 60 65 70 In considering the purely physical theory of

the results, the same can be readily explained. The invention may depend upon the defects of human vision in correctly analyzing color values. The whites cover a wide range of tints. Since a truly white object reflects white light waves without change in proportion to give the color "white", the added reflection of slightly more light of one color to give a tint, is not very noticeable. For example, the blue of the tint is merely an addition to the blue component of white light. In other words the amount of white which is present more or less blinds the eye to the tints. This is more true of blue than of yellow, because the eye is more sensitive to yellow. It is known that to the eye 15 a mixture of blue and yellow makes green. Since green is considered a restful color to the eye, the eye is not quick to note it, as it does yellow. It is therefore believed that the blue changes the reactions of the eye, by eliminating 20 the response it would get from yellow and substituting the less response it gets from green.

The foregoing physical theory is substantiated by the fact that any blue colors may be used, and by the old well known result of using blueing 25 in washing.

The invention may be used with diaotypes in general. There are two possible primary sources of yellowing in the background. One is the residue of the sensitizing substance after it is 30 decomposed by light. The other is residual coupling agents which may be in the paper or in the developer. It is known for a certainty that it may be one or both together which are culpable. It is recognized that the residual sensitizing solution may contain a phenolic substance. The coupling agents are commonly phenolic substances, and phenolic substances are discolored by light.

35 40 45 As set forth in the Van der Grinten patent the yellowing with age in light is a general characteristic of diaotypes, irrespective of the characters of the diazonium compound and of the coupling agents used. Upon these also depends the color of the pattern printed. The present invention is useful in place of the addition of the reducing agent of Van der Grinten, or as an addition to it.

The invention is of course not limited to the example given and such changes and modifications are intended as fall within the scope of the invention defined in the appended claims.

50 I claim:

55 1. A diaotype print having a commercially white back and face, the face having an additional blue tint not present in the back, the two whites being of such character that there is absence of sharp contrast between the face and the back, the said blue tint in the face serving to avoid a contrast between the face and the back upon aging of the print with the background of the face exposed to light.

60 65 70 75 80 85 90 95 2. A light-sensitive sheet comprising a white sheet coated on one side with a light-sensitive diazo composition with which is associated a blue coloring agent to give the coated side a blue component in its color, said blue color serving later in a diaotype made from said sheet to maintain a non-contrasting white appearance of the two faces under exposure to light sufficient to discolor to the eye the background of the print in the absence of such blue color.

WALKER M. HINMAN.